

UNITED STATES PATENT OFFICE.

PIERRE BERTHELEMY AND HENRY DE MONTBY, OF PARIS, FRANCE.

## PROCESS OF MANUFACTURING ALUMINUM ALLOY.

No Drawing. Application filed June 16, 1925, Serial No. 37,573, and in France May 11, 1925.

The present invention has for its subject a new aluminum alloy of which the density is substantially equal to that of aluminum itself, but of which the mechanical strength is much higher than that of aluminum. This alloy is essentially characterized by the fact that its composition includes copper, manganese, iron and silicon employed in the form of ferro-silicon, tungsten, magnesium, 10 also cadmium, and aluminum, in suitable determined proportions yielding a metal which may be subjected to any mechanical treatment (such as rolling, drawing, hammering, wire drawing and so forth, or even 15 cast and which in this case gives products free from cracks and flaws.

The invention also relates to the process of manufacture of the said alloy, according to which process there is first prepared a "rich alloy" of the body above specified by fusion in a plumbago crucible lined with magnesia and containing a certain quantity of a mixture of wood charcoal, calcium fluoride, oxide of magnesium and arsenous acid, the rich alloy thus produced being after scouring, run into ingot moulds for subsequent incorporation in aluminum in the proportion (variable according to the uses for which the metal is adapted) of 10 to 15 parts by weight of rich alloy to 90 to 85 parts by weight of aluminum.

Finally the invention has for its object a modification of the process, which modification is more particularly applicable in the case of alloys adapted to be fused, and in which the magnesium and cadmium (this latter body may be replaced by sodium) are only incorporated at the moment when the rich alloy is mixed with the aluminum, this incorporation being made at a temperature at most equal to  $725^{\circ}$  C.

With reference to examples which are given solely as examples of the methods of carrying the invention into effect, there will be described the method of preparation of alloys suitable for various uses. In all cases the rich alloy is prepared by fusing the constituents in a plumbago crucible lined with magnesia and in the bottom of which there are first placed 25 grammes of the following mixture:

The crucible is heated in a furnace permitting of obtaining a regular and constant temperature (heavy oil furnace or a furnace for heat recuperation of the Bigot system, for example). When the fusion has been effected, the alloy is agitated for a very long time by means of a rod of carbon from a retort lined with magnesia (a rod of iron should never be used for this operation). Then from the surface of the mass in fusion there is removed the mixture of powder and the slag which floats, which is run in small ingots in an ingot mould of iron lined with magnesia.

The composition of the rich alloy thus prepared varies according to the use to which the final alloy is adapted to be applied. 70

*Example 1.*—For obtaining an alloy adapted to form plates, rods, tubes, wires, sections and so forth, the rich alloy is prepared from the following substances: copper, 75 40 grammes; manganese, 2 grammes; ferro-silicon, 5.35 grammes, having 55% iron and 45% silicon (i. e. iron 3.95 gms., silicon 2.40 gms.); tungsten, 2 grammes; magnesium, 15 grammes; aluminum, 35.65 grammes. 80

The quantity of rich alloy obtained by fusing the preceding substances, in the manner indicated above, is incorporated in 900 grammes of pure aluminum (i. e. 99 to 99.5% pure). 85

*Example II.*—The rich alloy for the preparation of a meal adapted for the manufacture of castings of any nature, is obtained by fusing: copper, 42 grammes; manganese, 2 grammes; ferro-silicon, 5.35 grammes, having iron 55% and silicon 45% (i. e. iron 2.95 gms. and silicon 2.40 gms.); tungsten, 1 gramme; magnesium, 20 grammes; aluminum, 9.65 grammes.

The quantity of rich alloy thus obtained is incorporated in 900 grammes of pure aluminum. According to one essential feature of the invention, in this case particularly for the preparation of an alloy adapted for casting there are added, at the time of adding the rich alloy to the aluminum, 20 grammes of cadmium, this addition being for the purpose of eliminating cracks and flaws in the castings. 100 105

The magnesium which enters into the formulae of the rich alloys which have been indicated above (and also in the formula of the third example hereinafter set forth) may be added to the other constituents of the 110

|                           | Grammes. |
|---------------------------|----------|
| Pulverized beech charcoal | 1000     |
| Natural calcium fluoride  | 1000     |
| Oxide of magnesium        | 250      |
| 55 Arseneous acid         | 10       |

rich alloy and fused therewith, or it may be added, like the cadmium and at the same time as this metal, at the moment when the rich alloy is incorporated with the aluminum mass.

In all cases it is advisable, before adding these additions, to purify the metal, as otherwise there is the risk that the magnesium is drawn into the slag. On the other hand 10 it is essential to operate at a temperature which does not exceed 725° C. The fusion of the pure aluminum, with the incorporation of the appropriate rich alloy, is preferably effected in a plumbago crucible lined with magnesia and heated in an ordinary coke furnace.

The cadmium may be replaced by an equivalent quantity of sodium.

*Example III.*—A formula similar to the preceding is particularly suitable for the manufacture of engine pistons: copper, 52.50 grammes; manganese, 5 grammes; ferro-silicon, 5.50 grammes, having iron 55% and silicon 45% (i. e. iron 3.03 gms., and silicon 2.47 gms.); tungsten, 1 gramme; magnesium, 20 grammes; aluminum, 46 grammes.

This quantity of rich alloy is incorporated in 850 grammes of pure aluminum with the addition, under the conditions specified above, of 20 grammes of cadmium. The 20 grammes of magnesium called for by the formula of the rich alloy may be added at the same moment as the cadmium instead of being fused with the other constituents of 35 the rich alloy.

Irrespective of the formula adopted, it is important, in order to obtain products of good quality and constant characteristics, to use only pure metals and start with "cups" in the preparation of the rich alloys.

The metal adapted to be rolled should be previously heated for one hour at a temperature between 400 and 450° C. After two or 45 three rollings, the sheet should be re-heated under the same conditions, and this treatment is repeated until the required thickness is obtained. The sheet is then annealed at 450° C., and then immersed in a bath of hot water to which 5% of glycerine has been 50 added. Annealing can then be effected at a temperature of 450 to 475° C., and then the plate is allowed to cool slowly in air.

The manufacture of tubes, wires, rods, sections, is effected in the same manner.

Once the mechanical treatment has been completed, it is advisable to allow the metal to mature for from eight to ten days; and from this moment on it possesses all its permanent and desirable qualities.

Rapid artificial maturing of the castings (Examples II and III) can be promoted by subjecting them for one hour to annealing at a temperature of 200 to 250° C., which annealing is followed by immersion in a bath of boiling water to which 5% of glycer-

ine has been added. The same result is obtained by allowing the furnace to cool after annealing for one hour.

The aluminum alloy in the form of castings obtained according to the invention 70 can be readily tempered.

Having thus described our invention, what we claim as new and desire to secure by Letters Patent is:—

1. A process for the manufacture of an 75 aluminum alloy comprising fusing in a plumbago crucible lined with magnesia and containing a mixture of wood charcoal, calcium fluoride, oxide of magnesium, and arsenous acid, a mixture of copper, manganese, ferro-silicon, tungsten, magnesium, and aluminum, so as to produce a rich alloy, scouring the rich alloy, running the rich alloy into ingot moulds, and subsequently mixing the rich alloy with pure aluminum. 85

2. A process for the manufacture of an aluminum alloy comprising fusing in a plumbago crucible lined with magnesia and containing a mixture of wood charcoal, calcium fluoride, oxide of magnesium, and arsenous acid, a mixture of copper, manganese, ferro-silicon, tungsten, magnesium, and aluminum, so as to produce a rich alloy, scouring the rich alloy, running the rich alloy into ingot moulds, and subsequently 90 mixing the rich alloy with pure aluminum, in the proportion of 10 to 15 parts by weight of rich alloy to 90 to 85 parts by weight of aluminum. 95

3. A process for the production of an 100 aluminum alloy for the production of castings comprising fusing copper, manganese, ferro-silicon, tungsten, magnesium, and aluminum, in a plumbago crucible lined with magnesia and containing a mixture of wood charcoal, calcium fluoride, oxide of magnesium, and arsenous acid, the rich alloy thus obtained being scoured, run into ingot moulds, and then mixed with aluminum, and whilst mixing with the aluminum, adding magnesium and cadmium, this addition being made at a temperature of about 725° C. 110

4. A process for the production of an 115 aluminum alloy for the production of castings comprising fusing copper, manganese, ferro-silicon, tungsten, magnesium, and aluminum, in a plumbago crucible lined with magnesia and containing a mixture of wood charcoal, calcium fluoride, oxide of magnesium, and arsenous acid, the rich alloy thus obtained being scoured, run into ingot moulds, and then mixed with aluminum, and whilst mixing with the aluminum, adding magnesium and sodium, this addition being made at a temperature of about 725° C. 120

In witness whereof, we hereunto subscribe our names this 3rd day of June, 1925.

HENRY DE MONTBY.  
PIERRE BERTHÉLEMY.